

# United States Patent

[11] 3,540,663

[72] Inventor **John W. Dietz**  
Wilmington, Delaware  
[21] Appl. No. **725,151**  
[22] Filed **April 29, 1968**  
[45] Patented **Nov. 17, 1970**  
[73] Assignee **E. I. du Pont de Nemours and Company**  
Wilmington, Delaware  
a corporation of Delaware

[54] **MILLING OF METAL POWDERS IN THE  
PRESENCE OF IODINE**  
6 Claims, No Drawings

[52] U.S. Cl..... **241/22,**  
75/5, 75/213  
[51] Int. Cl. .... **B02b 5/02**  
[50] Field of Search..... **241/15, 16,  
17, 22, 30; 75/0.5, 0.5B.213**

[56]

## References Cited

### UNITED STATES PATENTS

|           |        |                    |        |
|-----------|--------|--------------------|--------|
| 1,703,634 | 2/1929 | Podszus.....       | 241/15 |
| 2,892,697 | 6/1959 | Davies et al. .... | 241/17 |
| 3,090,567 | 5/1963 | Schafer .....      | 241/22 |
| 3,252,842 | 5/1966 | Williams.....      | 241/16 |
| 3,301,494 | 1/1967 | Tornqvist .....    | 241/22 |

Primary Examiner—Gerald A. Dost  
Attorney—Norbert F. Reinert

**ABSTRACT:** Iodine is employed as a grinding aid in the milling of metal powders. Iodine is particularly useful in milling of metal powders to submicron sizes.

## MILLING OF METAL POWDERS IN THE PRESENCE OF IODINE

### BACKGROUND OF THE INVENTION

This invention relates to grinding aids for use in the milling of metal powders. Grinding aids are commonly used in the milling of metal powders to reduce reagglomeration of freshly milled particles, thereby reducing the milling time required and also lowering the minimum particle size that can be attained.

Organic acids, such as steric acid, and inorganic salts such as  $\text{Na}_2\text{Cr}_2\text{O}_7 \cdot 7\text{H}_2\text{O}$ ,  $\text{K}_3\text{Fe}(\text{CN})_6$  and  $(\text{NH}_4)_6\text{Mo}_7\text{O}_{24} \cdot 4\text{H}_2\text{O}$  are the most commonly used grinding aids. While these aids are relatively effective in preventing reagglomeration of very fine metal particles, they are difficult to remove once milling is complete. For example, if the organic acids are removed by heating, some decomposition will occur, leaving a residue of carbon and oxygen on the metal powder. Similarly, efforts to leach the inorganic salts from fine metal powders generally lead to oxidation of the metal.

This invention is founded on the discovery that iodine is superior to milling aids known to the art. More particularly, iodine is easy to handle; it is a solid at room temperature and can be weighed in the open air. More importantly, iodine is very effective in preventing reagglomeration of fine metal particles, inhibits oxidation of fine metal powders and can easily be removed by heating under vacuum.

### SUMMARY OF THE INVENTION

In summary, this invention is directed to the following: In a process for reducing the average particle diameter of metal powders comprising milling said powder in the presence of a grinding aid, the improvement wherein said grinding aid is iodine. This invention is also directed to submicron powders obtained by this process.

### DETAILED DESCRIPTION OF THE INVENTION

Although the mechanism whereby iodine improves the milling of metal powders is not clearly understood, it is believed that the iodine adsorbs on and reacts with the freshly formed metal surfaces. The surface coating thus formed is sufficiently adherent to prevent the reestablishment of direct metal-to-metal bonds whenever two surfaces are pressed tightly together during subsequent milling. It is to be understood, however, that the scope of this invention is not to be defined or limited in any manner by this theory.

The mill, milling fluid and milling medium used in practicing the method of this invention should be relatively unreactive toward iodine. Steel is a suitable construction material for the mill. Suitable milling fluids and milling media are discussed hereinafter.

While the amount of iodine used in the method of this invention can be varied considerably, it is preferable to use an amount which is sufficient to provide at least a monatomic layer on all surfaces of the final milled powder. Lesser amounts of iodine are not as effective but still provide considerable improvement in milling efficiency. Larger amounts of iodine do not greatly improve milling efficiency. In fact, a gross excess of iodine is very undesirable. The excess iodine may react with the metal powder, forming metal iodides and resulting in a substantial yield loss. In addition, if the amount of iodine present is sufficient to react with substantially all of the metal powder, then the reaction may proceed so vigorously as to cause the mill to erupt. For these reasons, it is desirable to limit the amount to less than the amount which will react with ten percent of the metal powder.

For the above-mentioned reasons, from 0.001 to 0.05 grams, and preferably from 0.005 to 0.02 grams, of iodine per square meter of surface area in the final metal powder will ordinarily be utilized.

There is only a practical upper limit on the particle size of the starting metal powder; this is about 40mesh. The method of this invention can be used to mill larger particles, but it is

ordinarily more convenient and economical to reduce the metal to minus 40-mesh, or somewhat less, by other methods known to the art. Preferably, minus 100-mesh powders are used as starting materials.

5 Iodine can be used as a grinding aid for those metals, or mixtures of metals, which are conventionally reduced to very fine powders by milling, e.g., scandium, yttrium, lanthanum, titanium, zirconium, hafnium, cerium, praseodymium, neodymium, promethium, samarium, europium, gadolinium, terbium, dysprosium, holmium, erbium, thulium, ytterbium, lutetium, vanadium, niobium, tantalum, chromium, molybdenum, tungsten, manganese, rhenium, iron, ruthenium, osmium, cobalt, rhodium, iridium, nickel, palladium, platinum, copper, silver, gold, aluminum, silicon and germanium.

10 15 Ballmilling is the conventionally preferred method of reducing the metal powders to submicron size. However, other milling procedures, such as air-attrition milling, can also be employed in practicing the method of this invention. The general rules of good milling practice should be followed in selecting the kind, size, and amount of milling media. A description of milling variables and the choice of optimum conditions is given in Chapter 16 of *Micromeritics*, J. M. DallaValle, Pitman Publishing Co., (New York 1934).

20 25 The milling media employed should be an abrasion-resistant material which has little or no reactivity toward iodine. Tungsten carbide bonded with cobalt is a preferred medium of this type. Another conventional milling medium is alumina. The milling media will ordinarily be spheres or cylinders whose

30 35 diameters and lengths are equal. The size of milling media should be at least ten times the initial particle size of the powder to be milled, but should not be appreciably greater than half an inch since this decreases milling efficiency. Optimum milling is generally obtained when the mill is filled approximately half full of media and the volume of powder and milling fluid is about equal to the volume of the voids in the milling media.

The mill should be completely enclosed or continuously purged with an inert gas so that moisture and oxygen cannot enter and react with the highly-reactive, fine metal powders. 40 As is customary in the art, it is ordinarily preferred to mill metal powders in an inert milling fluid, such as a light hydrocarbon oil. The oil helps protect the fine metal powder from oxidation, both during and after milling. The iodine coating also tends to protect the fine metal powder from oxidation. For this reason, it is often advantageous to leave the iodine coating on the metal powder even after milling is complete. In some instances, it will be most convenient to remove the iodine simultaneously with a subsequent processing step; for example, during the formation of sintered bodies from fine metal powders by heating in a vacuum or inert atmosphere, the iodine and metal iodide will sublime from the surface of the metal, leaving essentially no contamination in the product.

45 50 55 If it is desired to obtain a pure metal powder prior to subsequent processing, the iodine can be conveniently and completely removed by heating. Heating under vacuum is preferred since this permits the removal of the iodine at a lower temperature when sintering and grain growth are less likely to occur. Depending on the quality of vacuum employed, and on the particular metal being treated, the temperature required to effectively remove the iodine can vary from 20° to 600°C. Generally, 100° to 300°C. is most convenient.

60 65 70 The advantages of iodine as a grinding aid are particularly important when it is desired to produce metal powders having an average particle diameter of less than one micron. Such submicron metal powders are useful in the preparation of metal nitrides, carbides, phosphides, silicides, borides, etc. Incomplete reaction ordinarily results when coarser metal powders are utilized. Submicron metal powders are also used in mixtures with ceramics to form very strong composites or to form electrical resistance elements. Thus, the preferred products of the method of this invention consist of metal particles having at least a partial coating of iodine and having an

average diameter of less than one micron, as measured by conventional techniques for particle size counts on electron micrographs of fine powders. The preferred submicron powders of this invention are those having a surface area, by nitrogen adsorption, of at least one square meter per gram. The most preferred submicron powders of this invention are those having a surface area, by nitrogen adsorption, of at least four square meters per gram. The submicron powders of this invention are significantly less reactive toward atmospheric oxygen and nitrogen than are uncoated metal powders of the same surface area. The surface areas can be determined by the method described in "A New Method for Measuring the Surface Area of Finely Divided Materials and for Determining the Size of the Particles," by P. H. Emmett in symposium on New Methods for Particle Size Determination in the Subsieve Range, at the Washington Spring Meeting of ASTM, March 4, 1941.

*EXAMPLE 1*

180 Grams of minus 100-mesh titanium powder, 12 grams of iodine and 9,500 grams of  $\frac{1}{4}$ -inch by  $\frac{1}{4}$ -inch cylinders of cobalt-bonded tungsten carbide are placed in a 2.1-liter steel mill. Sufficient aliphatic hydrocarbon oil (b.p. 120-150°C.) is added to just cover the mixture. The mill is then closed tightly and rolled at approximately 75 revolutions per minute for 5 days.

The resulting slurry is washed from the mill and grinding cylinders with additional oil. The slurry is allowed to settle and the clear, supernatant oil is decanted. The residue is dried by heating to 100°C. in a glass resin kettle under an absolute pressure of 0.05 mm. of mercury for four hours. The sealed resin kettle is then transferred to a dry, nitrogen atmosphere where it is vented and the metal powder is removed. This metal powder is found to have a surface area, by nitrogen, adsorption, of  $5.0 \text{ m.}^2/\text{g.}$

*EXAMPLE 2*

100 Grams of minus 100-mesh aluminum powder, 10 grams of iodine and 1,800 grams of alumina balls  $\frac{1}{2}$ -inch in diameter are placed in a 2.1-liter steel mill. The mill is purged with argon and closed tightly. It is rolled at approximately 75 revolutions per minute for five days.

The mill is then transferred to a dry, nitrogen atmosphere where the product is separated from the alumina balls by screening through a 14-mesh screen. The metal powder is found to have a surface area, by nitrogen adsorption, of  $8.10 \text{ m.}^2/\text{g.}$

*EXAMPLE 3*

200 Grams of minus 40-mesh copper, 18 grams of iodine and 3,000 grams of  $\frac{1}{4}$ -inch by  $\frac{1}{4}$ -inch cylinders of cobalt-bonded tungsten carbide are placed in a 1.3-liter steel mill. Sufficient light aliphatic hydrocarbon oil (b.p. 130-150°C.) is added to cover the mixture. The mill is then closed and rolled at approximately 75 revolutions per minute for five days. The slurry is washed from the mill and dried as in Example 1. The resulting metal powder is found to have a surface area, by nitrogen adsorption, of  $1.8 \text{ m.}^2/\text{g.}$

I claim:

1. In a process for reducing the average particle diameter of a metal powder comprising milling said powder in the presence of a grinding aid, the improvement wherein said grinding aid is iodine.
2. The process of claim 1 wherein the amount of iodine utilized is sufficient to provide 0.001 to 0.05 grams per square meter of surface area of the product metal powder.
3. The process of claim 2 wherein the starting metal powder is minus 40-mesh and the product metal powder has an average particle diameter of less than one micron.
4. The process of claim 3 wherein said metal is titanium.
5. The process of claim 2 wherein the starting metal powder is minus 100-mesh and the product metal powder has an average particle diameter of less than one micron.
6. The process of claim 5 wherein said metal is titanium.

40

45

50

55

60

65

70

75